

## United States Patent Office

3,498,738

Patented Mar. 3, 1970

1

3,498,738

## REDUCING AGENT TREATMENT OF CROSS-LINKED CELLULOSIC TEXTILES HAVING A KETONE GROUP IN THE CROSS-LINK

Giuliana C. Tesoro, Dobbs Ferry, N.Y., assignor to J. P. Stevens &amp; Co., Inc., New York, N.Y., a corporation of Delaware

No Drawing. Filed Feb. 17, 1965, Ser. No. 433,510  
Int. Cl. D06m 1/02

U.S. Cl. 8-116

10 Claims

## ABSTRACT OF THE DISCLOSURE

Treatment of cellulosic materials containing carbonyl radicals with a reducing agent to improve the resistance of said material to hydrolysis in either an alkaline or acid medium.

This invention relates to a method for further modifying cellulosic materials containing carbonyl radicals and also relates to the cellulosic materials so modified. In particular, the invention relates to a method for treating cellulosic materials containing carbonyl radicals with a reducing agent.

In the growing field of technology concerned with chemical modification of cellulosic materials and especially textile forms such as yarn or fabric comprising cellulosic fibers, there have been substantial advances in the direction of introducing functional groups, which, in turn, have a marked effect on the physical and chemical properties of the cellulosic materials. One area of intensive study in this field relates to chemical modification of cellulosic textiles to impart crease-resistant and shape retentive properties. Another avenue of approach involves the introduction of polar radicals in order to impart additional desirable reactivity to the cellulose polymers.

Co-pending application Ser. No. 404,525, filed Oct. 16, 1964, now abandoned, entitled Process for Modifying Polymeric Materials and Modifier Reactants for Such Use, discloses the use of unique reactants for use in modifying cellulosic materials, among others. One class of the reactants described in the afore-mentioned application are ketones which react with the cellulose, thereby introducing carbonyl radicals. Di-functional ketone reactants having appropriate molecular structure are utilized to improve the crease recovery of cellulosic textile fabrics.

In addition to the foregoing, U.S. Patent No. 2,711,971 and U.S. Patent No. 3,109,695 describe methods of treating cellulosic textile fabrics to introduce carbonyl radicals into the cellulose polymer. British Patent No. 959,522 describes a process in which a cellulosic textile fabric is treated to introduce acrolein, a carbonyl radical containing substance.

In general, cellulosic materials modified by the introduction of carbonyl radicals by reaction of suitable carbonyl compounds with cellulosic polymers exhibit limited stability when exposed to various chemical substances of even moderate activity. For example, a white cotton textile fabric, modified by introduction of carbonyl radicals to impart wrinkle-resistance, becomes yellowed or discolored when subjected to repeated launderings. Such discoloration is due to the effect of exposure to alkaline conditions. It is obvious that such discoloration represents a severe disadvantage to the utility of carbonyl-containing chemicals which could otherwise be used for imparting wrinkle-resistance to cotton or cellulosic fabrics.

In addition to the above, cellulosic materials contain-

2

ing carbonyl radicals have poor resistance to hydrolysis in either acid or alkylne media. Thus, the improved properties obtainable as a result of the treatment of cellulosic materials with carbonyl-containing substances are not truly permanent in the sense that exposure of the cellulosic material to hydrolytic conditions may result in loss of properties due to loss of the carbonyl-containing substances or to other chemical changes.

In view of the foregoing, it is an object of the present invention to improve the stability of cellulosic materials which have been modified by introduction of carbonyl-containing substances.

It is a further object of this invention to improve the stability of cellulosic materials which have been modified by the introduction of carbonyl-containing radicals, by treatment thereof with a reducing agent.

It is another object of the present invention to stabilize cellulosic materials containing carbonyl radicals by treatment with reducing agents so that the cellulosic polymers are substantially unaffected by exposure to hydrolytic conditions.

Another object of the present invention is to substantially eliminate discoloration by laundering of cellulosic materials which have been treated to introduce carbonyl-containing substances.

Briefly stated, one embodiment of the present invention is a method of treating a cellulosic material containing carbonyl radicals which comprises the step of treating the said cellulosic material with a reducing agent having sufficient reducing power to convert at least a substantial portion of the carbonyl radicals to a reduced form.

As indicated above, there are many prior art processes involving treatment of cellulose or cellulose-containing materials with carbonyl-containing substances in order to impart improved properties. The present invention is intended to encompass all such modified cellulosic material regardless of the nature of the carbonyl-containing substance and the specific manner of introduction thereof. In addition, the present invention does not distinguish between materials formed exclusively from cellulose, such as a cotton fabric, and those which contain cellulosic polymers in addition to others. The latter class includes, for example, a fabric composed of cotton and polyester fibers.

Since carbonyl radicals are not easily reduced, it is necessary to choose reducing agents which have substantially strong reducing power. The alkali borohydrides are typical of the preferred reducing agents suitable for use in the present invention. This class of materials includes sodium borohydride ( $NaBH_4$ ); potassium borohydride ( $KBH_4$ ) and lithium borohydride ( $LiBH_4$ ).

Application of the reducing agent to the carbonyl-containing cellulosic material can be accomplished by any convenient method. Thus, the cellulosic material can be immersed in a solution containing the reducing agent or, alternatively, the cellulosic material may be padded or sprayed with a solution containing the reducing agent. Although any inert solvent may be utilized to prepare the solution containing the reducing agent, aqueous solutions are preferred because of the simplicity of the operation and from the stand-point of cost.

As is well known, the solubility and reactivity of reducing agents may be dependent on the pH of the environment. (See Melland Textilber, 44, August 1963, pp. 839-843.) Certain reducing agents such as the alkali borohydrides are more effective at a relatively high pH, of the order of 10 or more; whereas others such as morpholine borane are preferably utilized at a relatively

low pH, of the order of 2. The formula for morpholine borane, which is a member of the general class of amino boranes, is as follows:



The reduction of carbonyl radicals with alkali borohydrides can be implemented by the use of certain inorganic salts which act as catalysts or accelerators. This phenomenon is disclosed in U.S. 3,118,724. Such catalysts or accelerators include complex metal salts of copper, nickel and cobalt, and magnesium, aluminum and lithium halides.

The effect of treatment of carbonyl-containing cellulosic materials in accordance with the present invention can be analytically determined by analysis of the change in carbonyl content. From a practical stand-point, the improvement obtained by treatment in accordance with the present invention may be obtained by results of tests such as the following:

(1) Decrease in the weight loss resulting from exposure to hydrolytic conditions.

(2) Absence of discoloration after exposure to conditions which would otherwise cause discoloration.

(3) Improved stability to hydrolytic conditions determined from measurement of physical properties.

Set forth below are examples which are intended to illustrate the process of the present invention. As can be seen, the cellulosic materials, following treatment, are superior to the control samples.

The standard tests utilized in the following examples are referenced as set forth below:

(1) Carbonyl content: (A) H. Stübchen-Kirchner, Oesterr. Chem. Z. 61 132 (1960); (B) U. Ströle, 1. Europa Symposium Darmstadt, 1958

(2) Crease recovery: ASTM-D1295-60T

(3) Reflectance: ASTM-E97-55 (green, tristimulus filter)

#### EXAMPLE 1

Samples of 80 x 80 cotton print cloth were modified with bis (2-pyridinium ethyl) ketone dichloride according to the following procedure.

The cloth was impregnated with an aqueous solution of the ketone dichloride using a laboratory padder. The cloth was then framed and dried at 60° C., treated with an aqueous sodium hydroxide solution, saturated with sodium chloride and maintained in a flat condition for about one minute. The cloth was then rinsed successively with dilute acetic acid, water and acetone and finally washed thoroughly in a dilute non-ionic detergent solution. The cloth was then framed and dried.

hydride solution was varied as indicated in the table below.

A control sample of the ketone dichloride modified cloth was analyzed and was found to have a weight gain of 4.75% and a carbonyl radical content of 0.92 weight percent.

Set forth below in tabular form are the results of this experiment, showing the percent carbonyl content and the crease recovery of the various samples.

|    |         |                       |      | Percent decrease in CO content | Percent decrease in CO content | Crease recovery (degrees W+F) |
|----|---------|-----------------------|------|--------------------------------|--------------------------------|-------------------------------|
|    |         | Duration of reduction |      | Dry                            | Wet                            |                               |
| 15 | Sample: |                       |      |                                |                                |                               |
|    | A       | None                  | 0.92 | 190                            | 252                            |                               |
|    | B       | 10 minutes            | 0.42 | 55                             | 206                            | 266                           |
|    | C       | 30 minutes            | 0.36 | 61                             | 198                            | 256                           |
|    | D       | 1 hour                | 0.33 | 64                             | 199                            | 251                           |
| 20 | E       | 3 hours               | 0.23 | 75                             | 199                            | 252                           |
|    | F       | 6 hours               | 0.11 | 88                             | 207                            | 250                           |

It may be seen that the crease recovery properties of the ketone modified cloth are not affected by the reduction of the carbonyl radical content.

Samples A through F were exposed to alkaline hydrolytic conditions by immersion in a 0.5 N sodium hydroxide solution for a period of about 3 hours. The alkaline solution was maintained at about 65° C. and a fabric-liquid weight ratio of about 1 to 50 was used. Sample A lost a significant proportion of the increase in weight attributable to the ketone dichloride treatment. In addition, sample A took on a yellow color and exhibited a loss in crease recovery.

For samples B and C, the extent of the discoloration, loss in weight and loss in crease recovery represented an improvement over sample A.

Samples D, E and F remained white in color, lost substantially no weight and showed substantially no decrease in crease recovery.

#### EXAMPLE 2

Samples of 80 x 80 cotton print cloth were modified with bis(2-pyridinium ethyl)ketone dichloride in accordance with the method outlined in Example 1. These samples were treated by immersion in an aqueous solution of sodium borohydride, maintained at about 50° C. Four solutions were used. Each of the solutions contained sodium hydroxide in the concentrations indicated in the table below. In addition, the concentration of the reducing agent and time of reduction were varied. As noted, two of the solutions contained cyanide accelerators.

The results of this experiment were as follows:

| Reducing solution                       | Catalyst added                           | Time of reduction | Percent CO |
|-----------------------------------------|------------------------------------------|-------------------|------------|
| (1) None                                |                                          |                   | 1.2        |
| (2) 5% NaBH <sub>4</sub> in 0.5N NaOH   | None                                     | 2 hours           | 0.1        |
| (3) 0.5% NaBH <sub>4</sub> in 0.2N NaOH | do                                       | 15 minutes        | 0.35       |
| (4) 0.5% NaBH <sub>4</sub> in 0.2N NaOH | 0.02% K <sub>2</sub> CO(CN) <sub>6</sub> | do                | 0.20       |
| (5) 0.5% NaBH <sub>4</sub> in 0.2N NaOH | 0.02% K <sub>2</sub> Ni(CN) <sub>6</sub> | do                | 0.20       |

Samples of the cloth, modified as above, were treated with a reducing agent in the following manner. The samples were immersed in a solution of 0.3% by weight sodium borohydride in isopropanol solution, the solution being maintained at a temperature of about 50° C. The duration of exposure of the samples to the sodium boro-

#### EXAMPLE 3

Samples of 80 x 80 cotton print cloth were modified with di-hydroxy acetone in accordance with the general procedure described in U.S. 3,109,695. The samples were found by analysis to have exhibited a weight gain of 9.2% and had a carbonyl radical content of 1.5 weight percent.

Samples as described above were treated with sodium borohydride by immersion in a solution thereof. The fabric to solution ratio was 1 to 50. The specific conditions of each of the experimental runs was as follows:

| Conc. of reducing agent percent by weight | Solvent                            | Temperature of solution °C | Duration of reduction, hours | Percent decrease CO |
|-------------------------------------------|------------------------------------|----------------------------|------------------------------|---------------------|
| (1) 0.3                                   | Isopropanol                        | 50                         | 3                            | 19                  |
| (2) 0.3                                   | do                                 | 55                         | 5                            | 23                  |
| (3) 4                                     | Tetraethylene glycol dimethylether | 80                         | 3                            | 42                  |
| (4) 8                                     | Dimethyl formamide                 | 80                         | 5                            | 42                  |

The samples tested in accordance with runs 3 and 4 exhibited relatively high resistance to both acid and alkaline hydrolytic conditions.

#### EXAMPLE 4

Samples of 80 x 80 cotton print cloth were modified with acetone-formaldehyde precondensate in accordance with the general procedure in U.S. 2,711,971. The samples were found by analysis to have a weight gain of 10.2% and a carbonyl content of 1.1%.

Samples modified as above, were immersed in an aqueous solution containing 5% sodium borohydride and 0.02%  $K_2Ni(CN)_4$ . The solution contained sodium hydroxide in an amount to provide the 0.2 N solution. The fabric to solution ratio was 1 to 50. The solutions were maintained at 65° C.

Set forth below are the results of these experiments:

| Sample: | Reduction time, hours | Percent CO content |     | Percent decrease of CO content |
|---------|-----------------------|--------------------|-----|--------------------------------|
|         |                       | None               | 1.1 |                                |
| A       | 1                     | 0.17               | 85  |                                |
| B       | 3                     | 0.20               | 82  |                                |
| C       | 6                     | 0.18               | 84  |                                |

After reduction, the samples were exposed to alkaline hydrolysis by treating with a 1 N aqueous NaOH solution for 3 hours at 65° C. (fabric to solution ratio of 1 to 50). After hydrolysis, the following results were obtained:

| Sample: | Crease Recovery |     |       |     | Loss of reflectance after hydrolysis, percent |   |
|---------|-----------------|-----|-------|-----|-----------------------------------------------|---|
|         | Before          |     | After |     |                                               |   |
|         | Hydrolysis      | Dry | Wet   | Dry |                                               |   |
| A       | 29              | 264 | 260   | 208 | 216                                           | 8 |
| B       | 4               | 256 | 250   | 249 | 231                                           | 0 |
| C       | 5               | 255 | 238   | 251 | 228                                           | 0 |
| D       | 4               | 251 | 237   | 255 | 236                                           | 0 |

It is apparent that unreduced sample A was discolored (as shown by the loss of reflectance), and lost resilience (as shown by the loss in crease recovery) while the reduced samples B, C and D were unchanged after the hydrolytic treatment.

#### EXAMPLE 5

Samples of 80 x 80 cotton print cloth were modified with acetone-formaldehyde precondensate in accordance with the general procedure described in U.S. 2,711,971. Upon analysis, the samples were found to have a weight gain of 8.3% and a carbonyl content of 1.2%.

A first aqueous solution, solution A, was made up to contain 5.0 weight percent of sodium borohydride and sufficient sodium hydroxide to provide a 0.2 N concentration. A second aqueous solution, solution B, was made up to contain the same amount of sodium hydroxide and sodium borohydride as solution A and contained, in addition, 0.2%  $K_2Ni(CN)_4$ .

The samples were treated with the respective solutions using a laboratory padder. Following impregnation of the samples, they were exposed to super-heated steam at a temperature in the range of from about 100°-110° C. in

a laboratory steamer for a period of about 5 minutes. The steamed samples were rinsed in succession with 1% acetic acid solution, water and were then washed thoroughly in non-ionic detergent solution, maintained at 50° C. The samples were framed and dried. The following results were obtained:

| Reducing solution: | Percent CO |
|--------------------|------------|
| None               | 1.2        |
| Solution A         | 0.32       |
| Solution B         | 0.31       |

The unreduced and the reduced samples were exposed to alkaline hydrolysis (2 N NaOH at the reflux temperature for 3 hours, fabric-solution ratio 1 to 50), and the following changes were noted as a result of the reducing treatment:

| Sample           | Crease Recovery (W+F) Dry |                  | Loss of reflectance percent |
|------------------|---------------------------|------------------|-----------------------------|
|                  | Before hydrolysis         | After hydrolysis |                             |
| Not reduced      | 215                       | 190              | 13                          |
| Treated w/Sol. A | 225                       | 218              | 2                           |
| Treated w/Sol. B | 220                       | 209              | 1                           |

#### EXAMPLE 6

Samples of 80 x 80 cotton print cloth were modified with acetone formaldehyde precondensate in accordance with Example 4 of U.S. 2,711,971. One group of samples, designated Sample A, was found by analysis to have a weight gain of 15.4% and a carbonyl content of 1.5%. Another group of samples, designated Sample B, was found by analysis to have a weight gain of 10.2% and a carbonyl content of 1.1%.

Samples as described above were immersed in an aqueous solution of morpholine borane of 5 weight percent. Sufficient sulfuric acid was added to the solution to give a pH of about 1.5. The solution was maintained at a temperature of about 60° C, and the samples were immersed for about 5 hours, the fabric to solution ratio being 1 to 50.

Set forth below are the results:

| Sample: | Percent CO Reduction |        | Percent decrease of CO content | Percent loss of added weight |
|---------|----------------------|--------|--------------------------------|------------------------------|
|         | Percent wt. gain     | Before |                                |                              |
| A       | 15.4                 | 1.5    | 0.8                            | 47                           |
| B       | 10.2                 | 1.1    | 0.7                            | 36                           |

It can be seen that a substantial reduction in carbonyl content can be obtained without significant overall weight loss.

#### EXAMPLE 7

Samples of 80 x 80 cotton print cloth were modified with acetone formaldehyde precondensate in accordance with the general procedure disclosed in U.S. 2,711,971. The samples so treated were found upon analysis to have a weight gain of 7.8% and a carbonyl content of 1.1%.

Samples, treated as above, were impregnated with an aqueous solution containing 1% by weight of sodium borohydride and sufficient sodium hydroxide to provide a concentration of 0.2 N. The impregnation was accomplished by use of a laboratory padder. One set of samples, Sample A, was exposed to super-heated steam at a temperature of 100°-110° C. for a period of two minutes in a laboratory steamer. Another set of samples, Sample B, was dried in a laboratory forced air oven at a temperature of 95° C. for a period of about 5 minutes.

Both sets of samples were successively rinsed with 1% acetic acid solution and water and were then thoroughly washed in a non-ionic detergent solution, maintained at a temperature of 50° C. The samples were then framed and dried. The results of this experiment were as follows:

| Sample      | Percent CO | Percent decrease of CO content | Tensile (W) <sup>1</sup> after 10 launderings | Tear (W) <sup>2</sup> after 10 launderings |
|-------------|------------|--------------------------------|-----------------------------------------------|--------------------------------------------|
| Not reduced | 1.1        |                                | 35                                            | 1.1                                        |
| A           | 1.14       | 76                             | 42                                            | 1.2                                        |
| B           | 0.16       | 88                             | 40                                            | 1.1                                        |

<sup>1</sup> Tested according to strip method, ASTM-D-39-59.

<sup>2</sup> Tested according to Elmendorf method, ASTM-D-1424-59.

All of the above samples were then exposed to alkaline hydrolytic conditions, i.e., an aqueous 2 N sodium hydroxide solution, for a period of three hours at a temperature of about 100° C. Set forth below are the values of crease resistance and reflectance, measured both before and after exposure of the samples to hydrolytic conditions.

| Sample      | Crease Resistance |        | Reflectance |       |
|-------------|-------------------|--------|-------------|-------|
|             | Dry (W+F)         | Before | Before      | After |
| Not reduced | 268               | 207    | 87          | 71    |
| Reduced A   | 243               | 223    | 86          | 81    |
| Reduced B   | 248               | 235    | 87          | 80    |

In addition to the reducing agents utilized in the above example, other materials which are suitable for use in the invention include:



Morpholine borane, the use of which is described in one of the examples above, is typical of the group of amino boranes which are generally suitable as reducing agents in the present invention. The formula for amino boranes is as follows:



In general, reducing agents which can be used for practicing the process of the present invention are those having an  $r_H$  value lower than about +1,  $r_H$  value being defined as the negative logarithm of the equilibrium hydrogen pressure over the solution of reducing agent (see Melland Textilber 44, p. 839, 1963).

The concentration of reducing agent required to obtain the desired result is dependent upon the carbonyl content of the cellulosic material to be treated and is also dependent upon the activity of the particular reducing agent selected. In general, concentrations in the

range of about 0.5% to 5% by weight in the treating solution are effective.

Of course, the usual reaction parameters which affect reducing reactions also apply in the present invention. Thus, for example, the temperature utilized must be considered, although temperatures in the wide range up to 150° C. give satisfactory results.

The present invention has been shown to substantially increase the utility of cellulosic materials which have previously been treated to introduce carbonyl radicals. In general, the carbonyl content of the cellulosic material is of little consequence and likewise, the manner in which the carbonyl radical is introduced in the cellulosic material is of minor importance. The process of the present invention is applicable regardless of whether the cellulosic materials are side chain modified or whether they are cross-linked. It is immaterial whether the cellulosic materials have been reacted with carbonyl containing radicals in the presence of alkaline or acidic catalysts or whether reacted in the presence of swelling agents or in their absence.

The cellulosic materials which are suitable for treatment in accordance with the present invention may be composed wholly or in part of natural cellulose such as cotton, and regenerated cellulose such as rayon or cellophane film. The cellulosic materials may also include linen, flax and the like.

The physical shape and character of the cellulosic materials which are amenable to treatment by the present invention include such well known forms as film, fiber, yarn and fabric.

What has been described above is a process for modifying the characteristics of cellulosic materials which have been previously treated to incorporate carbonyl radicals. It has been shown by use of examples that the treatment of the present invention which involves use of a reducing agent stabilizes the cellulosic materials in question and eliminates certain undesirable properties. It is to be understood that the examples are merely illustrative and changes in the process as described may be made by one skilled in the art.

What is claimed is:

1. The method of treating a crosslinked cellulosic textile material containing dimethylene ketone or diethylene ketone crosslinks which comprises treating said crosslinked textile material with a solution comprising a reducing agent having a  $r_H$  value below about +1,  $r_H$  being defined as the negative logarithm of the equilibrium hydrogen pressure over the solution of the reducing agent.

2. The method of treating a crosslinked cellulosic textile material containing dimethylene ketone or diethylene ketone crosslinks which comprises treating said crosslinked textile material with a solution comprising an alkali borohydride as a reducing agent.

3. The method of claim 2 wherein said reducing agent is sodium borohydride.

4. The method of treating a crosslinked cellulosic textile material containing dimethylene ketone or diethylene ketone crosslinks which comprises treating said crosslinked textile material with a solution comprising an amino borane.

5. The method of claim 4 wherein said reducing agent is morpholino borane.

6. The method of treating a cellulosic textile material which has been crosslinked with a formaldehyde-acetone condensation product having up to 4 methylo groups per mol of acetone which comprises treating said crosslinked textile material with a solution comprising a reducing agent having a  $r_H$  value below about +1,  $r_H$  being defined as the negative logarithm of the equilibrium hydrogen pressure over the solution of the reducing agent.

7. The method according to claim 6 wherein said reducing agent is an alkali borohydride.

8. The method of claim 7 wherein said reducing agent is sodium borohydride.

9. The method according to claim 6 wherein said reducing agent is an amino borane.

10. The method of claim 9 wherein said reducing agent is morpholino borane.

References Cited

UNITED STATES PATENTS

|           |        |                   |       |           |
|-----------|--------|-------------------|-------|-----------|
| 2,898,333 | 8/1959 | Jullander         | ----- | 8—107 X   |
| 3,017,316 | 1/1962 | Rapson            | ----- | 8—108.5 X |
| 3,032,548 | 5/1962 | Jullander         | ----- | 8—107 X   |
| 3,043,719 | 7/1962 | Burr et al.       | ----- | 8—116.3 X |
| 3,198,651 | 8/1965 | Shiraishi         | ----- | 8—108 X   |
| 3,318,657 | 5/1967 | Wade              | ----- | 8—107 X   |
| 3,341,279 | 9/1967 | Fregermuth et al. | ----- | 8—116 X   |

FOREIGN PATENTS

610,655 12/1960 Canada.

OTHER REFERENCES

5 Meller, TAPPI, vol. 36, No. 8, pp. 366—367 (1953).  
 Meller, TAPPI, vol. 38, No. 11, pp. 682—687 (1955).  
 Nevell et al., Journal of the Textile Institute, vol. 53,  
 T90—T93 (1962).

10 GEORGE F. LEMES, Primary Examiner  
 J. CANNON, Assistant Examiner  
 U.S. Cl. X.R.  
 15 8—107, 133; 260—232

UNITED STATES PATENT OFFICE  
CERTIFICATE OF CORRECTION

Patent No. 3,498,738 Dated March 3, 1970

Inventor(s) Giuliana C. Tesoro

It is certified that error appears in the above-identified patent and that said Letters Patent are hereby corrected as shown below:

Column 2, line 2, "alkyline" should read --alkaline--.  
Column 3, line 14, "cobalt" should read --cobalt--; line 40, "tristimulu" should read --tristimulus--. Column 4, lines 60-65, in the table, line (2), "NaOh" should read --NaOH--. Column 6, line 51, "perecnt" should read --percent--; line 60, in the table, the caption for the third and fourth columns should read:

| <u>Percent CO</u> |              |
|-------------------|--------------|
| <u>Before</u>     | <u>After</u> |
| <u>Reduction</u>  |              |

Column 7, line 22, in the table, second column, "1.14" should read --0.14--.

SIGNED AND  
SEALED

SEP 29 1970

(SEAL)

Attest:

Edward M. Fletcher, Jr.

Attesting Officer

WILLIAM E. SCHUYLER, JR.  
Commissioner of Patents